

G. H. GROCE AND G. M. HOWARD,  
ANODE FOR ELECTROLYTIC RECTIFIERS,  
APPLICATION FILED AUG. 17, 1920.

1,436,709.

Patented Nov. 28, 1922.



INVENTORS  
George H. Groce and  
George M. Howard  
BY  
Lyman E. Dodge  
ATTORNEY

Patented Nov. 28, 1922.

1,436,709

# UNITED STATES PATENT OFFICE.

GEORGE H. GROCE, OF CHICAGO, ILLINOIS, AND GEORGE M. HOWARD, OF PHILADELPHIA, PENNSYLVANIA.

## ANODE FOR ELECTROLYTIC RECTIFIERS.

Application filed August 17, 1920. Serial No. 404,049.

*To all whom it may concern:*

Be it known that we, GEORGE H. GROCE and GEORGE M. HOWARD, both citizens of the United States, the former a resident of Chicago, county of Cook, State of Illinois, the latter a resident of Philadelphia, county of Philadelphia, State of Pennsylvania, have invented certain new and useful Improvements in Anodes for Electrolytic Rectifiers, 5 set forth in the following specification.

This invention relates to anodes for electrolytic rectifiers.

The principal object of this invention is an improvement in an anode for an electrolytic rectifier, which will result in longer 15 life of that anode.

Other objects and advantages will appear as the description of the invention progresses, and the novel features of the invention will be particularly pointed out in 20 the appended claims.

In describing the invention in detail, reference is had to the accompanying drawing wherein has been illustrated a preferred 25 physical embodiment of the invention, and wherein like characters of reference designate corresponding parts throughout the several views, and in which:

Figure 1 is a longitudinal cross sectional 30 view of an anode constructed in accordance with the invention; and Fig. 2 is an end view of the device illustrated by Fig. 1.

The anode of electrolytic rectifiers is generally constructed of lead or polished steel. 35 Although theoretically it may be that the anode should not dissolve or disintegrate in use, nevertheless in practice the anode wears away quite rapidly. In order to obviate this defect the present invention provides

40 that the current carrying portion of the electrode wherein contact with the electrolyte shall consist of an alloy of lead and antimony and preferably one containing not less than about eight per centum of antimony 45 by weight.

The electrode may be made in various forms but it is preferred to make the electrode in the form illustrated by the drawing accompanying and forming a part of this 50 application.

In the preferred form shown by the drawing, the member 3 is the electrode composed of an alloy of lead and antimony, containing preferably not less than about 55 eight per centum of antimony by weight.

Electrodes of the same size and run for the same length of time and at the same current density gave on test the following loss in weight with different materials: pure lead 6.7%; 4% antimony 0.8%; 8% antimony 60 0.04%. Still higher percentages of antimony were tried but no advantage over the 8% antimony was found.

In the preferred form the electrode 3 is surrounded by a tube 4, formed of a material not acted upon by the electrolyte of an electrolytic rectifier. This tube 4 is preferably formed of metal and is best formed of steel.

The electrode 3 is held in the tube 4 and 70 spaced therefrom by insulating material 5 and 6. This insulating material is preferably cork and is positioned as shown so as to make a liquid tight joint both at point of contact with the tube and with the electrode, 75 both at the upper end and at the lower end.

In practice the current conducting wire is connected to the top of the rod 3 and the electrode is immersed in an electrolyte of suitable composition to such an extent that 80 the electrolyte does not reach the top of the tube 4 as shown by top surface 7 of an electrolyte so that no electrolyte comes in contact with the electrode at the surface line 85 of the electrolyte.

Although the construction of one physical embodiment of the invention has been particularly described, and the operation and principle thereof explained, nevertheless, it is desired to have it understood that 90 the form selected is merely illustrative, but does not exhaust the possible physical embodiments of the idea of means underlying the invention.

What we claim and desire to secure by 95 United States Letters Patent is:

1. In an electrolytic rectifier, in combination: an electrode composed of an alloy of lead and antimony containing not less than about eight per centum by weight of antimony.

2. In an electrolytic rectifier an electrode which has all parts in contact with an electrolyte which carry current composed of an alloy of lead and antimony containing not 105 less than about eight per centum of antimony by weight.

GEORGE H. GROCE.  
GEORGE M. HOWARD.